# EUROPEAN PATENT SPECIFICATION

(11) **EP 0 664 746 B1**
(45) Date of publication and mention of the grant of the patent: **19.02.1997**
(21) Application number: 93921049.8
(22) Date of filing: 04.10.1993
(51) Int. Cl.: B44C 1/17, D06Q 1/14, D06P 5/00

(54) **APPLIQUE AND METHOD FOR ITS MANUFACTURE**
ABZIEHBILD UND VERFAHREN ZU DESSEN HERSTELLUNG
APPLIQUE ET PROCEDE DE FABRICATION

(30) Priority: 17.10.1992 GB 9221945
(43) Date of publication of application: 02.08.1995
(73) Proprietor: FABREX LIMITED, Hinckley Leicestershire LE10 1AW (GB)
(72) Inventor: ENGLAND, Douglas Roy, Lutterworth, Leics LE17 5BB (GB)
(74) Representative: Hallam, Arnold Vincent
(86) International application number: GB9302055
(87) International publication number: WO9408799

(56) References cited:
- EP-A- 0 312 299
- GB-A- 2 066 158
- GB-A- 2 126 951
- GB-A- 2 243 332
- US-A- 4 292 100

## Description

The present invention relates to appliqués.

Known appliqués generally comprise one or more layers of material, of which the uppermost layer of material is a thermoplastics material film on which a design is printed. Such appliqués are intended for bonding to a substrate, normally an item of clothing, by heat and high frequency welding. Appliqués are normally manufactured in sheet form with the appliqué printed design being repeated a dozen or more times on the sheet before the sheet is separated into individual appliqués. One of the major problems associated with the use of thermoplastics material is that it has a low elasticity level and when stretched, although it will try and revert to its previous state, it does not entirely succeed and thus becomes distorted after stretching. This results in distortion of the printed design. During multicoloured printing of a sheet of appliqués, the thermoplastics material moves or stretches slightly when each colour impression is made, as a result of which it is impossible to print large sheets with the colours exactly in register over the whole sheet. In addition, the inks used in printing normally need to be cured at 160°C or higher. However, the thermoplastics material used in the manufacture of appliqués has a melting point of typically between 180°C and 200°C and begins to distort at 150°C, causing distortion of the appliqué after printing.

GB-A-2 243 332 describes a printing method which includes an ink image forming step and an ink image transferring step. In the ink image forming step, an ink image is formed on a hot-melting type adhesive layer of a transfer sheet by using a heat-sensitive image transfer type recording device. In the image retransferring step, the ink image and the hot-melting type adhesive layer are transferred onto an image receiving member such as a cloth by heatedly pressing the transfer sheet.

EP-A-0 312 299 discloses a transfer element which is adapted to be applied to an article in face-up orientation by mechanical means. The transfer element comprises a base or carrier on which is supported a release layer of thermoplastic material, an intermediate support layer, a pattern or design superimposed on the support layer, a second support layer applied over the pattern or design, and a cover coat of an adhesive material. The transfer is applied by raising its temperature to a temperature causing the release layer to melt and the cover coat to become tacky whereby the cover coat, design, support layers and a portion of the release layer may be separated from the base or carrier and applied to the surface of an article, the temperatures of the release layer and cover coat being controlled so that they attain a state whereby the degree of adherence of the release layer to the surface of the article exceeds the degree of adherence of the cover coat to the transfer member, so that the latter may be withdrawn leaving the transfer adhered to the surface of the article.

The present invention seeks to provide an improved appliqué and method of manufacture.

Accordingly, the present invention provides a method of manufacturing an appliqué comprising:
providing a laminate of a first layer comprising a thermoplastics material, and a second layer of a substrate material for supporting said thermoplastics material during printing;
and printing a preselected design on an upper surface of said first layer;
wherein prior to the step of printing said preselected design said laminate is passed through a blind printing cycle, said blind printing cycle being a printing cycle for the laminate in which no printing ink is used and no design is therefore printed on the laminate.

The use of a "blind printing cycle" has the effect of preparing and stabilising the thermoplastics material layer with the result that when a design is subsequently printed on the laminate a lower distortion of the design occurs and, when two or more colour impressions are made, a much better registration of the coloured inks with one another is obtained.

The present invention also provides an appliqué comprising a laminate having:
a first layer comprising a thermoplastics material;
and a second layer of a substrate material serving to support said thermoplastics material during printing of a preselected design on said first layer;
wherein the substrate contains polyester and polyamide fibres.

In a preferred form of the invention the substrate is a silicone material conveniently having a nominal weight of 180gsm. Alternatively or additionally, the substrate may be a paper with a silicone coating or layer.

The thermoplastics material is conveniently PVC and the substrate provides a stable base for the PVC, restricting movement of the PVC in varying ambient temperatures, varying states of "wetness" during printing and varying humidity conditions. The substrate also enables the PVC to retain its normal state at a temperature above 150°C during curing of the printing inks, when it would normally begin to distort. As a result, it provides a stable base for inks to be cured at a temperature of between 150°C and 200°C and preferably between 165°C and 185°C.

### Example 1

In one example of appliqué according to the present invention, a thermoplastics material layer, 0.2mm thick is supported on a substrate 0.2mm thick and is coated with an adhesive layer to which flock is secured. The flock has a fibre content which is dispersed at a rate of 100g per m², compared with a normal rate of 80g per m². The fibres are also cut at 0.5mm length with the fibre having a weight of typically 1.7g/10Km of fibre (1.7 desitex).

The substrate has the following parameters which are average production values:

| **Parameter** | **Unit** | **Test Method** | **Values** |
|---|---|---|---|
| Weight | g/m² | DIN 53 104 | 170 |
| Thickness | mm | DIN 53 105 | 0.190 |
| Density | g/m³ | DIN 53 105 | 0.9 |
| Tensile MD | N | DIN 53 112 | 160 |
| CD | | | 110 |
| Elongation MD | % | DIN 53 112 | 3 |
| CD | | | 5 |
| Smoothness (Bekk) | | DIN 53 107 | 20 |
| Water absorbtion (Cobb) | | DIN 53 132 | 15 |

Advantageously, the adhesive layer is 0.125mm thick to enable the root of each fibre to contact the thermoplastics material layer, leaving 0.375mm of each fibre exposed.

The maximum thickness of the printed appliqué is about 1mm, preferably 0.9mm.

The control of the flock enables the printing process to be much more exacting since the improved density and uniformity of height of the flock fibres more closely resembles a flat surface. The "blind printing cycle" also has the effect of removing rogue fibres i.e. extra long fibres protruding above the finished flock surface.

During printing, the improved density and pressure equalisation created by the uniform height of the fibres reduces surface movement of the fibres when the weight and pressure of a printing screen is introduced onto the flock surface. The surface more closely resembles a flat stable surface producing a clear print.

The ink used in printing the design on the thermoplastics material is a water-based ink which contains a thickening agent (typically Sericol ZE596) and a flock transfer catalyst (typically Sericol FT386), these preferably being added at 5% and 6% by weight, respectively. The thickener also enables ink to be deposited directly onto the flock itself without "bleeding" i.e. without the ink leaking away from the printed areas. The use of a catalyst and thickening agent improves the viscosity of the ink to aid deposit of the ink and render it less transparent. It also reduces the curing temperature of the ink and enables the ink to bond better to the flock.

The ink curing process is effected using a dryer such as a gas dryer at a constant temperature of 165°C to 185°C for two to three minutes.

Printing can be effected to a resolution equivalent to 11.8 dots pro mm (300dpi.)

Each printing ink colour is left to dry after curing for between one and three hours in ambient temperature to avoid any unnecessary movement of the thermoplastics material layer and after the final printing the appliqués are left to dry in atmosphere overnight. Alternatively, drying can be effected in wicket dryers at a suitable temperature above ambient, e.g. up to 40°C.

The percentage elongation of the finished product (substrate, PVC and flock) is compared below with the substrate itself, and with the PVC and flock layer without the substrate support.

| | Wet Elongation % | |
|---|---|---|
| | MD | CD |
| (a) Stable Substrate | 0.15 | 0.30 |
| (b) S.S./PVC/Flock (finished product) | 0.10 | 0.17 |
| (c) PVC & Flock | 0.55 | 0.10 |
| MD = Machine Direction CD = Cross Direction | | |

Finally, during welding of an appliqué according to the present invention to an item of clothing, an impervious film of acetate may be sandwiched between the appliqué and the article of clothing to prevent migration of ink between the two.

## Claims

1. A method of manufacturing an appliqué comprising:
providing a laminate of a first layer comprising a thermoplastics material, and a second layer of a substrate material for supporting said thermoplastics material during printing;
and printing a preselected design on an upper surface of said first layer;
wherein prior to the step of printing said preselected design said laminate is passed through a blind printing cycle, said blind printing cycle being a printing cycle for the laminate in which no printing ink is used and no design is therefore printed on the laminate.

2. A method as claimed in claim 1 wherein said substrate comprises paper with a silicone layer thereon.

3. A method as claimed in claim 1 wherein said substrate comprises a silicone material.

4. A method as claimed in claim 2 or wherein said substrate has a weight of substantially 180g per m² .

5. A method as claimed in any of the preceding claims wherein said substrate contains polyester and polyamide fibres.

6. A method as claimed in any of the preceding claims wherein said thermoplastics material is PVC.

7. A method as claimed in any of the preceding claims wherein said thermoplastics material has a layer of flock adhered thereto to form said upper surface of said first layer.

8. A method as claimed in claim 7 wherein said flock has a density of 100g per m².

9. A method as claimed in claim 7 or 8 wherein said flock is formed from fibres having a length of substantially 0.5mm.

10. A method as claimed in claim 7, 8 or 9 wherein said flock comprises fibres havinga weight of 1.7g/10Km of fibre (1.7 desitex).

11. A method as claimed in any of the preceding claims wherein said substrate has a maximum elongation of 5% when tested according to DIN 53 112.

12. A method as claimed in any of the preceding claims wherein said preselected design is printed using a water-based ink.

13. A method as claimed in claim 12 wherein said ink contains a thickening agent and a flock transfer catalyst.

14. A method as claimed in claim 13 wherein said thickening agent forms approximately 5% by weight of said ink and said flocker transfer catalyst forms approximately 6% by weight of said ink.

15. A method as claimed in any of the preceding claims wherein the step of printing said preselected design comprises:
a) printing a first coloured ink on said upper surface of said first layer;
b) curing said ink at a temperature in the range 165° to 185° for a preselected time period;
c) allowing said ink to dry in ambient temperature for a second preselected time period; and
repeating steps (a) to (c) for each further coloured ink.

16. A method as claimed in claim 15 wherein said first preselected time period is in the range two to three minutes and said second preselected time period is in the range one to three hours.

17. An appliqué comprising a laminate having:
a first layer comprising a thermoplastics material;
and a second layer of a substrate material serving to support said thermoplastics material during printing of a preselected design on said first layer;
wherein said substrate contains polyester and polyamide fibres.

18. An appliqué as claimed in claim 17 wherein said substrate comprises paper with a silicone layer thereon.

19. An appliqué as claimed in claim 17 wherein said substrate comprises a silicone material.

20. An appliqué as claimed in claim 18 or 19 wherein said substrate has a weight of substantially 180g per m².

21. An appliqué as claimed in any of the preceding claims wherein said thermoplastics material is PVC.

22. An appliqué as claimed in any of the preceding claims wherein said thermoplastics material has a layer of flock adhered thereto to form said upper surface of said first layer.

23. An appliqué as claimed in claim 22 wherein said flock has a density of 100g per m².

24. An appliqué as claimed in claim 22 or 23 wherein said flock is formed from fibres having a length of substantially 0.5mm.

25. An appliqué as claimed in claim 23, 24 or 25 wherein said flock comprises fibres having a thickness of 1.7 desitex.

26. An appliqué as claimed in any of the preceding claims wherein said substrate has a maximum elongation of 5% when tested according to DIN 53 112.

27. An appliqué as claimed in any of the preceding claims wherein said preselected design is printed using a water-based ink.

28. An appliqué as claimed in claim 26 wherein said ink contains a thickening agent and a flock transfer catalyst.

29. An appliqué as claimed in claim 27 or 28 wherein said thickening agent forms approximately 5% by weight of said ink and said flocker transfer catalyst forms approximately 6% by weight of said ink.

## Patentansprüche

1. Eine Vorgangsweise der Herstellung einer Applikationsarbeit, bestehend aus:
der Vermittlung eines Laminats aus einer ersten Schicht, bestehend aus einem thermoplastischen Material und einer zweiten Schicht eines Substrats zum Tragen besagten thermoplastischen Materials während des Druckvorgangs;
und Drucken eines festgelegten Designs auf die Oberfläche besagter erster Schicht;
wobei vor dem Vorgang des Druckens besagten festgelegten Designs besagtes Laminat einen Blinddruck durchläuft, wobei es sich um einen Druckzyklus für das Laminat handelt, in dem keine Druckerfarbe zur Verwendung kommt, weshalb kein Design auf das Laminat aufgedruckt wird.

2. Eine Vorgangsweise nach Anspruch 1, wobei besagtes Substrat auf Papier mit darauf befindlicher Silikonschicht besteht.

3. Eine Vorgangsweise nach Anspruch 1, wobei besagtes Substrat aus einem Silikonmaterial besteht.

4. Eine Vorgangsweise nach Anspruch 2, wobei besagtes Substrat ein Gewicht von größtenteils 180 g/m² hat.

5. Eine Vorgangsweise nach einem der o.g. Ansprüche, wobei besagtes Substrat Polyester- und Polyamidfasern enthält.

6. Eine Vorgangsweise nach einem der o.g. Ansprüche, wobei besagtes thermoplastisches Material PVC ist.

7. Eine Vorgangsweise nach einem der o.g. Ansprüche, wobei besagtes thermoplastisches Material eine darauf aufgezogene Flockfaserschicht hat, die besagte Oberfläche besagter erster Schicht bildet.

8. Eine Vorgangsweise nach Anspruch 7, wobei besagte Flockfaser eine Dichte von 100 g/m² hat.

9. Eine Vorgangsweise nach Anspruch 7 oder 8, wobei besagte Flockfaserschicht aus Fasern gebildet ist, die eine Länge von größtenteils 0,5 mm haben.

10. Eine Vorgangsweise nach Ansprüchen 7, 8 oder 9, wobei besagte Flockfasern ein Gewicht von 1,7 g/10 km Faserlänge haben (1,7 Desitex).

11. Eine Vorgangsweise nach einem der o.g. Ansprüche, wobei besagtes Substrat bei Prüfung nach DIN 53 112 eine maximale Dehnung von 5% hat.

12. Eine Vorgangsweise nach einem der o.g. Ansprüche, wobei besagtes festgelegtes Design mit einer Druckerfarbe auf Wasserbasis gedruckt wird.

13. Eine Vorgangsweise nach Anspruch 13, wobei besagte Druckerfarbe ein Verdickungsmittel und einen Flocktransferkatalyst enthält.

14. Eine Vorgangsweise nach Anspruch 13, wobei besagtes Verdickungsmittel ungefähr 5 Gewichtsprozent und besagter Flocktransferkatalyst ungefähr 6 Gewichtsprozent besagter Druckerfarbe ausmacht.

15. Eine Vorgangsweise nach einem der o.g. Ansprüche, wobei der Schritt des Druckens besagten festgelegten Designs folgendes umfasst:
a) Drucken einer ersten farbigen Druckerfarbe auf besagte Oberfläche besagter erster Schicht;
b) Härten besagter Druckerfarbe für einen festgelegten Zeitraum bei einer Temperatur im Bereich von 165 bis 185°;
c) Trocknen besagter Druckerfarbe für einen weiteren Zeitraum bei Raumtemperatur; und
Wiederholen von Schritten (a) bis (c) für jede weitere bunte Druckerfarbe.

16. Eine Vorgangsweise nach Anspruch 15, wobei besagter erster festgelegter Zeitraum im Bereich von zwei bis drei Minuten und besagter zweiter festgelegter Zeitraum im Bereich von einer bis drei Stunden liegt.

17. Eine Applikationsarbeit, bestehend aus einem Laminat mit
einer erste Schicht, bestehend aus einem thermoplastischen Material;
und einer zweiten Substratschicht, die besagtes thermoplastisches Material während des Druckens eines festgelegten Designs auf besagte erste Schicht trägt;
wobei besagtes Substrat Polyester- und Polyamidfasern enthält.

18. Eine Applikationsarbeit nach Anspruch 17, wobei besagtes Substrat Papier mit einer darauf befindlichen Silikonschicht umfasst.

19. Eine Applikationsarbeit nach Anspruch 17, wobei besagtes Substrat ein Silikonmaterial umfasst.

20. Eine Applikationsarbeit nach Ansprüchen 18 oder 19, wobei besagtes Substrat ein Gewicht von größtenteils 180 g/m² hat.

21. Eine Applikationsarbeit nach einem der o.g. Ansprüche, wobei besagtes thermoplastisches Material PVC ist.

22. Eine Applikationsarbeit nach einem der o.g. Ansprüche, wobei besagtes thermoplastisches Material eine damit verbundene Flockfaserschicht hat, die besagte Oberfläche besagter erster Schicht bildet.

23. Eine Applikationsarbeit nach Anspruch 22, wobei besagte Flockfaser eine Dichte von 100 g/m² hat.

24. Eine Applikationsarbeit nach Anspruch 22 oder 23, wobei besagte Flockfaser aus Fasern mit einer Länge von größtenteils 0,5 mm besteht.

25. Eine Applikationsarbeit nach Ansprüchen 23, 24 oder 25, wobei besagte Flockfaser aus Fasern mit einer Dicke von 1,7 Desitex besteht.

26. Eine Applikationsarbeit nach einem der o.g. Ansprüche, wobei besagtes Substrat bei Prüfung nach DIN 53 112 eine maximale Dehnung von 5 % hat.

27. Eine Applikationsarbeit nach einem der o.g. Ansprüche, wobei besagtes festgelegtes Design mit einer Druckerfarbe auf Wasserbasis gedruckt wird.

28. Eine Applikationsarbeit nach Anspruch 26, wobei besagte Druckerfarbe ein Verdickungsmittel und einen Flocktransferkatalyst enthält.

29. Eine Applikationsarbeit nach Ansprüchen 27 oder 28, wobei besagtes Verdickungsmittel ungefähr 5 Gewichtsprozent und besagter Flocktransferkatalyst ungefähr 6 Gewichtsprozent besagter Druckerfarbe ausmacht.

## Revendications

1. Une méthode de fabrication d'un appliqué, comportant:
création d'un stratifié d'une première couche comportant une matière thermoplastique et d'une seconde couche d'un substrat pour supporter ladite matière thermoplastique pendant l'impression;
et impression d'un motif présélectionné sur une surface supérieure de ladite première couche;
méthode selon laquelle, avant l'étape d'impression du dit motif présélectionné, ledit stratifié est soumis à un cycle d'impression à vide, ledit cycle d'impression à vide étant un cycle d'impression pour le stratifié durant lequel aucune encre d'impression n'est utilisée et aucun motif n'est donc imprimé sur le stratifié.

2. Une méthode selon la revendication 1, dans laquelle ledit substrat comporte du papier recouvert d'une couche de silicone.

3. Une méthode selon la revendication 1, dans laquelle ledit substrat comporte une matière au silicone.

4. Une méthode selon la revendication 2, dans laquelle ledit substrat a un poids substantiel de 180 g/m².

5. Une méthode selon l'une quelconque des revendications précédentes, dans laquelle le substrat contient des fibres de polyester et de polyamide.

6. Une méthode selon l'une quelconque des revendications précédentes, dans laquelle ladite matière thermoplastique est du PVC.

7. Une méthode selon l'une quelconque des revendications précédentes, dans laquelle de la matière à floquer est collée sur ladite matière thermoplastique pour former ladite surface supérieure de ladite première couche.

8. Une méthode selon la revendication 7, dans laquelle ladite matière à floquer possède une densité de 100 g/m².

9. Une méthode selon la revendication 7 ou 8, dans laquelle ladite matière à floquer est constituée à partir de fibres d'une longueur substantielle de 0,5 mm.

10. Une méthode selon la revendication 7, 8 ou 9, dans laquelle ladite matière à floquer comporte des fibres d'un poids de 1,7 g/km de fibre (1,7 desitex).

11. Une méthode selon l'une quelconque des revendications précédentes, dans laquelle ledit substrat présente un allongement maximum de 5% lorsque éprouvé selon DIN 53 112.

12. Une méthode selon l'une quelconque des revendications précédentes, dans laquelle ledit motif présélectionné est imprimé à l'aide d'une encre à base d'eau.

13. Une méthode selon la revendication 12, dans laquelle ladite encre contient un agent épaississeur et un catalyseur de transfert de matière à floquer.

14. Une méthode selon la revendication 13, dans laquelle ledit agent épaississeur forme environ 5% du poids de ladite encre et ledit catalyseur de transfert de matière à floquer forme approximativement 6% du poids de ladite encre.

15. Une méthode selon l'une quelconque des revendications précédentes, dans laquelle l'étape d'impression du dit motif présélectionné comporte:
a) impression d'une première encre colorée sur ladite surface supérieure de ladite première couche;
b) séchage de ladite encre à une température dans la plage de 165° à 185° pendant une durée présélectionnée;
c) séchage de ladite encre à la température ambiante pendant une seconde durée présélectionnée; et
reprise des étapes (a) à (c) pour chaque autre encore colorée.

16. Une méthode selon la revendication 15, dans laquelle ladite première période présélectionnée se situe dans la plage de deux à trois minutes et ladite seconde période présélectionnée se situe dans la plage de une à trois heures.

17. Un appliqué comportant un stratifié possédant:
une première couche comportant une matière thermoplastique;
et une seconde couche d'un substrat servant à supporter ladite matière thermoplastique pendant l'impression d'un motif présélectionné sur ladite première couche;
dans lequel ledit substrat contient des fibres de polyester et de polyamide.

18. Un appliqué selon la revendication 17, dans lequel ledit substrat comporte du papier recouvert d'une couche de silicone.

19. Un appliqué selon la revendication 17, dans lequel ledit substrat comporte une matière au silicone.

20. Un appliqué selon la revendication 18 ou 19, dans lequel ledit substrat pèse substantiellement 180 g/m².

21. Un appliqué selon l'une quelconque des revendications précédentes, dans lequel ladite matière thermoplastique est du PVC.

22. Un appliqué selon l'une quelconque des revendications précédentes, dans lequel une couche de matière de flocage est collée sur ladite matière thermoplastique pour former ladite surface supérieure de ladite première couche.

23. Un appliqué selon la revendication 22, dans lequel ladite matière de flocage possède une densité de 100 g/m².

24. Un appliqué selon la revendication 22 ou 23, dans lequel ladite matière de flocage est formé de fibres d'une longueur substantielle de 0,5 mm.

25. Un appliqué selon les revendications 23, 24 ou 25, dans lequel ladite matière de flocage comporte des fibres d'une épaisseur de 1,7 desitex.

26. Un appliqué selon l'une quelconque des revendications précédentes, dans lequel ledit substrat présente un allongement maximum de 5% lorsque éprouvé selon DIN 53 112.

27. Un appliqué selon l'une quelconque des revendications précédentes, dans lequel ledit motif présélectionné est imprimé avec une encre à base d'eau.

28. Un appliqué selon la revendication 26, dans lequel ladite encre contient un agent épaississeur et un catalyseur de transfert de matière de flocage.

29. Un appliqué selon la revendication 27 ou 28, dans lequel ledit agent épaississeur forme environ 5% du poids de ladite encre et ledit catalyseur de transfert de matière de flocage forme environ 6% du poids de ladite encre.
